

# UNITED STATES PATENT OFFICE.

BOTHO SCHWERIN, OF FRANKFORT-ON-THE-MAIN, GERMANY, ASSIGNOR TO ELEKTRO-OSMOSE AKTIENGESELLSCHAFT (GRAF SCHWERIN GESELLSCHAFT), OF FRANKFORT-ON-THE-MAIN, GERMANY, A CORPORATION.

## PROCESS FOR REMOVING LIQUID FROM STEATITE.

1,266,330.

Specification of Letters Patent.

Patented May 14, 1918.

No Drawing. Application filed November 11, 1914, Serial No. 871,626. Renewed October 24, 1917. Serial No. 198,260.

*To all whom it may concern:*

Be it known that I, BOTHO SCHWERIN, a subject of the German Emperor, residing at Frankfort-on-the-Main, Germany, have invented certain new and useful Improvements in Processes for Removing Liquid from Steatite, of which the following is a specification.

The present invention relates to a process for removing of water from steatite by electro-osmosis. The invention relates particularly to a process by which, without increasing the consumption of energy a considerable increase in the degree of dryness can be achieved in respect to the methods now known.

It has been found, that the electro-osmotic removal of water becomes the more effective the more finely subdivided the material is; that is to say, as the smallness of the particles increases the extent to which the water is removed and the rapidity of the osmosis increase. The present improvement, therefore, consists in comminuting the steatite to as finely subdivided condition as possible before subjecting it to the electro-osmotic process for removing water. The degree of fineness is limited by commercial considerations.

In the chemical treatment of colloids the effect is frequently enhanced by adding to the colloidal body or to a suspension thereof, an electrolyte suitable for bringing the body into the condition of a colloidal solution (sol-condition).

Hitherto the proportion of the added electrolyte has been determined in relation either to the volume or the weight of the substance to which it is to be added. This rule generally leads to unfavorable results since the permissible maximum of added electrolyte is exceeded and the effect thereby diminished. I have found, that the maximum permissible addition of electrolyte does not depend on the quantity and the weight of the solid part or on the volume of the liquid in which it is suspended, but the most favorable addition of electrolyte depends on the superficies of the dispersoid, that is to say, under otherwise equal conditions on the degree of dispersion of the solid body.

Thus is the further object of this invention to bring the degree of comminution

into such relationship with the amount of added electrolyte, that the maximum of addition for a given degree of dispersion is attained. Here also the limit depends on commercial conditions, namely cost of comminution and cost of electrolyte.

When a body to be comminuted, such as steatite, is subjected to the operation in presence of the electrolyte, the latter has the effect of rendering the comminution much more rapid and thorough. The body is to a certain degree opened up by the electrolyte. This favorable action is of further importance, since, as already stated, the more electrolyte that can be added the greater the degree of dispersion of the solid substance. In this manner there is obtained a considerable increase in the dehydrating effect per unit time and in the content of dry substance in the finished material.

I have found, that the favorable effect of adding an electrolyte is not experienced or only incompletely experienced in the case of many materials. The effect of the electrolyte can now be considerably increased by adding to the mass a colloid body in addition to an electrolyte. Such bodies are, for instance, colloidal silicic acid, humic acid, organic and inorganic colloids. By adding bodies of this kind the effect of the electrolyte is increased. The colloidal body may be added to the mass before the electrolyte is added, or simultaneously therewith.

For example, in the treatment of steatite an addition of sodium silicate produces favorable results. In this case the colloid body (colloidal silicic acid) and the suitable electrolyte are united. The former is liberated by hydrolysis and adsorbed, whereas the alkali constitutes the electrolyte.

If, in the treatment of steatite, sodium silicate is added, the silicic acid freed through hydrolysis is adsorbed by the steatite and remains adsorbed. The behavior in this case of the colloidal substances added to the electrolyte outside of the steatite depends upon the fact that these highly charged colloidal substances are adsorbed by the steatite and so function directly against the action of the electrolyte.

The sodium silicate is dissociated in water partly into sodium hydroxid and silicic acid (hydrolysis). The silicic acid is adsorbed

by the steatite though it is not certain whether as ortho-, metha-, or poly-silicic acid. The sodium hydroxid represents the electrolyte.

5 The silicic acid adsorbed from the steatite is present in extraordinarily small masses so that the steatite is obtained in an almost chemically pure condition. These small particles of silicic acid do no harm as the steatite itself is a magnesium silicate.

10 What I claim, is:

15 1. In a process for removing water from steatite, finely subdividing the steatite in the presence of an electrolyte suitable for bringing the solid body into sol-condition and subjecting the steatite to the electro-osmotic treatment.

2. In a process for removing water from steatite, finely subdividing the steatite in the presence of an electrolyte suitable for bringing the solid body into sol-condition, and of a colloid body, and subjecting the steatite to the electro-osmotic treatment. 20

3. In a process for removing water from steatite subdividing the steatite in the presence of sodium silicate and subjecting the steatite to the electro-osmotic treatment. 25

In testimony whereof I affix my signature in presence of two witnesses.

BOTHO SCHWERIN.

Witnesses:

JEAN GRUND,  
CARL GRUND.